

## UNITED STATES PATENT OFFICE

1,985,718

BITUMINOUS PAVING MATERIAL AND  
METHOD OF PRODUCING THE SAME

James F. Carle, Birmingham, Ala.

No Drawing. Application July 15, 1931,  
Serial No. 551,059

8 Claims. (Cl. 106—31)

My invention relates to a process of manufacture and laying of bituminous pavements. It particularly relates to improvements in bituminous paving or surfacing compositions which may be readily stored, handled, transported and laid while cold, and to the processes and methods of manufacturing the same. It also relates to similar compositions which are preferably reheated immediately before being laid.

10 The primary object of this invention is to effect greater economy and utility in the manufacture and use of bituminous paving compositions.

A more specific object of the invention is the production of a bituminous mixture in a loose granular state which may be handled and stored cold and which may be laid and compacted into a dense, tough and durable pavement by the application of pressure, with or without a preliminary heating.

20 In the production of bituminous compositions intended to be stored, handled and transported cold, certain serious and well defined difficulties and limitations have been encountered either or both as to the selection of bituminous materials and gradings of mineral aggregates and as to their utility as paving materials. These difficulties have heretofore increased the cost of such compositions and limited their use for the most part to light or medium traffic pavements 25 and to patchwork and small jobs where the increased cost of the cold mixture is less than the cost of installing local mixing plants and other facilities for the manufacture and laying of standard hot mixtures.

30 In the practice of the present invention I am able to produce cold paving compositions in an economical manner from substantially all standard combinations and gradings of mineral aggregates and mineral fillers as now commonly specified for standard types of bituminous pavements, such as sheet asphalt, stone filled sheet asphalt, asphaltic concrete of the fine and coarse aggregate types, including binders, and so-called black bases of the asphaltic concrete type, and 35 for treating and utilizing bituminous sandstone and limestone, using standard commercial grades of bitumens, or asphaltic cements, without the use of volatile solvents, liquefiers, or other special ingredients or treatments of the bituminous or asphaltic material before mixing.

It is understood that properly fluxed native or other hard asphalts may be used, as well as a small amount of volatile solvents if desired for special purposes, but these are not essential to the process. The use of volatile solvents and

fluxes containing a substantial percentage of volatile constituents is in general to be avoided as tending to produce an inferior product. It is understood also that variations from standard gradings of mineral aggregates and percentages of mineral fillers may be used.

For mixtures which are to be laid cold, softer asphalts or bitumens having a higher penetration are used than those commonly specified for mixtures of corresponding types which are laid 10 hot. For example, asphalts that are of sufficiently high penetration to be plastic at atmospheric temperatures should be employed. As in general a slightly lower percentage of total bitumen is used in the mixture than is commonly 15 used in mixtures of the same type which are to be laid hot.

The essential features of the process of producing bituminous compositions of the character herein disclosed, and which is claimed to 20 be new and useful, consists in the manner and combination of treatments of the heated bituminous composition immediately after it has been mixed in the conventional manner, and comprises the various steps in sequence, separately and in combination with each other, which 25 have for their purpose the granulation of the composition as a whole and particularly the substantial toughening and stabilizing of the immediate surfaces of the bituminous coating on the 30 individual particles of the mineral aggregates.

To illustrate clearly the technical and scientific principles involved, reference is made first to the well known toughening and stabilizing effect of certain specific mineral fillers, as for example, when finely ground limestone is incorporated into the body of bituminous materials, it exhibits high absorptive and surface tension effects with relation to the bituminous substances. As illustrative of this high absorptive and surface 35 tension effect, it has been discovered that powdered lime, when sprinkled into a solution of asphalt in benzol, chloroform and similar solvents will remove the asphalt from the solution causing it to precipitate as separate particles each comprising a lime nucleus surrounded by the asphalt. Similarly, it has been found that powdered lime 40 will remove asphalt from emulsions thereof.

I have discovered after extensive investigation with bituminous materials that when such materials are introduced into a water suspension of hydrated lime, finely ground limestone and similar basic and substantially insoluble materials, that a thin continuous film of the suspended substance is readily formed or adsorbed on the sur- 50 55

face of bituminous material. This coating serves to render the bituminous surfaces non-sticky, within substantial ranges of pressure and temperature, and prevents the coalescence of different particles or surfaces with each other.

Accordingly, the various steps and sequence of treatments, comprising my improved process have been developed which when carried out with proper relation to each other and of temperature, 10 produce a cooled and granulated composition in a wet or moist condition in which the immediate external surfaces of bituminous coatings are provided with a thin continuous toughened film of sufficient stability to prevent the setting up of 15 the mixture under all normal conditions of handling and storage, but leaving the body of the bituminous coatings sufficiently plastic at atmospheric temperatures to permit the composition to be readily consolidated into a stable and 20 durable pavement under pressure as in rolling or tamping.

For the purpose of forming the protective coating, finely ground material or inorganic substance containing a high percentage of the oxides, hydroxides, carbonates, or basic silicate of calcium and such magnesium as ordinarily accompanies limestone or dolomite, including bituminous limestone and basic blast furnace slags have been found to be efficient. It is understood that other 25 similar neutral or basic substances may be used, but clays and all substances which have a preferential absorption for water or which exhibit emulsifying properties or tendencies as between bituminous materials and water, are especially 30 excluded as tending to produce inferior products. Only substances are selected which possess the 35 property of being readily adsorbed by bituminous surfaces from water suspensions, and which also act as effective fillers or stabilizers of the bituminous composition when consolidated into the 40 final pavement.

In the manufacture of the improved bituminous composition I take sand or suitable combinations of fine and coarse aggregates which are 45 usually selected approximately in accordance with standard gradings and specifications for standard type of bituminous surfaces, binders or base courses and heat same until thoroughly dry and at a suitable temperature for mixing with bituminous materials which will ordinarily be found 50 to be from 150° to 350° F., depending on the character of the bituminous material used. The heated aggregate either with or without the addition of mineral filler is mixed with the asphalt cement or bituminous material, which is also heated until in a liquid condition, in a pug mill or other suitable mixing device.

If necessary the remaining steps of the process 55 may be completed in the same pug mill or mixing device, but owing to the time required and other disadvantages it is preferable to discharge the mixed material immediately into a separate cooling and mixing device. For this purpose a trough conveyor of sufficient length and capacity to hold 60 several batches from the mixer may be used. This conveyor is suitably provided with a revolving shaft having blades or paddles which are set at a suitable angle so as to force the bituminous mixture slowly forward while retaining it in a 65 comparatively loose condition. On being discharged into the trough conveyor the heated loose mixture is immediately sprayed with cold water at one or more points in sufficient amount to 70 thoroughly wet and partially cool the mixture.

75 At a selected point along the length of the

conveyor, where the temperature has been reduced to around the softening point of the asphaltic or bituminous material, or to approximately 140° F., and the mixture thoroughly granulated by the action of the mixing blades, a quantity of finely divided mineral or inorganic material above described is added to the mixture either in a dry state or in the form of a suspension in cold water. For this purpose I have found that a suspension of hydrated lime 10 is preferable, though satisfactory results may be obtained with powdered limestone and other materials heretofore mentioned. In case bituminous limestone is used it is preferably added dry. Additional water is added and as the material is 15 further mixed and conveyed forward a thin coating is formed on the surface of the bituminous films covering the particles or pieces of aggregate.

In treating the coated aggregate with the suspension of finely divided calcareous material, care 20 must be exercised to partially cool the coated aggregate down to near the softening point of the asphalt. If treated at too high a temperature, the high absorptive power and surface tension of the calcareous material is such that it 25 may partially remove the coating from the aggregate.

It has been found that the coatings are formed chiefly from the finer particles of pulverized material and most of the coarser particles and any 30 excess material is finally drained or washed away with the excess cooling water. Usually, the finished product will contain from one to three per cent of the fine coating material, depending on the kind of material used and the character of 35 the mixture. The mixture may be discharged from the conveyor directly into stock piles but if not cooled to a point substantially below the softening point of the bituminous material used it may first be discharged into cold water. Due 40 to the great affinity of the calcareous materials adsorbed into the surface of the bituminous material, the discharging into cold water or subsequent washing does not remove the adsorbed surface coating. The particles thus treated remain in a loose separate condition until subjected to compressive action such as by rolling or tamping when the material is laid in a pavement.

It is especially pointed out that when bituminous compositions prepared as herein described 50 are conveyed to stock piles, the excess water rapidly drains away but a small percentage of moisture is held tenaciously for a long period of time, and this fact is an important part of the process as a contributing factor in retaining the composition in a workable condition. It has been found, however, that the completely dried material will remain in storage for many months without showing any substantial tendency to bond or set up into an unworkable mass.

The material thus treated is in especially good condition for laying in a pavement and, unless the harder grades of asphalt are employed, requires no preliminary heating before being spread and rolled upon the roadway. The compressive 65 and kneading action on the particles when rolled forces the inner layers of bituminous materials through the outer coating of each particle and bonds it to adjacent particles, while the calcareous coating material, due to its great surface tension and absorptive power for the bituminous materials acts as a filler thereby toughening and increasing the stability of the pavement.

While I have described my invention in but one form it will be obvious to those skilled in 75

the art that it is not so limited, but is susceptible of various changes and modifications without departing from the spirit thereof, and I desire, therefore, that only such limitations shall be placed thereupon as are imposed by the prior art or as are specifically set forth in the appended claims. Also while I have described my improved product as being applicable to paving material, it will be obvious that it may be used for other purposes where a dense tough and durable material is required.

What I claim is:—

1. A process of producing a mixed bituminous material adapted to be stored in a granular condition and laid cold and to solidify upon compression, comprising, mixing hot bituminous material of sufficiently high penetration to be plastic at atmospheric temperatures with granular aggregate, maintaining said mixture in a granular condition by agitation, providing a water suspension of finely divided calcareous material, partially cooling the mixture while maintaining it in a granular condition and treating the granular bituminous material with said water suspension at a temperature near the softening point of the bituminous material.

2. A process of producing bituminous paving material adapted to be stored in a granular condition and laid cold and to solidify upon compression, comprising, mixing bituminous binder material of sufficiently high penetration to be plastic at atmospheric temperatures with granular aggregate, agitating with disintegration to maintain the mixture in a granular condition, providing a water suspension of finely divided calcareous material, treating the granular bituminous material while agitating with said water suspension at a temperature near the softening point of the bituminous material, and discharging the materials thus treated into cold water.

3. A process of producing bituminous paving material adapted to be stored in a granular condition and laid cold and to solidify upon compression, comprising, mixing bituminous material of sufficiently high penetration to be plastic at atmospheric temperatures with granular aggregate at a temperature of from 150° to 350° F., stirring the mixed substance to maintain it in a granular condition, cooling the granular mixture until it is at a temperature near the softening point of the bituminous material, and treating it while in a granular condition with a water suspension of finely divided calcareous material.

4. A process of producing bituminous paving

material adapted to be stored in a granular condition and laid cold and to solidify upon compression, comprising mixing heated bituminous material of sufficiently high penetration to be plastic at atmospheric temperatures with heated granular aggregate, partially cooling and stirring the mixed materials to maintain them in a granular condition, and applying a coating of finely divided calcareous material to the granular particles when at a temperature near the softening point of the bituminous material.

5. A process of producing bituminous paving material adapted to be stored in a granular condition and laid cold and to solidify upon compression, comprising, mixing bituminous material of sufficiently high penetration to be plastic at atmospheric temperatures with granular aggregate heated to a temperature of from 150° to 350° F., partially cooling and stirring the mixed materials to maintain them in a granular condition, applying a coating of finely divided calcareous material to the granular particles when at a temperature near the softening point of the bituminous material, and discharging the coated granular material into cold water.

6. A ready mixed bituminous road material adapted for storage in a loose condition and to be compacted into a solidified mass upon the application of pressure, consisting in mineral aggregate covered with a bituminous binder of sufficiently high penetration to be plastic at atmospheric temperatures, and the latter having a coating of adsorbed finely divided calcareous material.

7. A ready mixed road paving material adapted for storage in a loose condition and to be compacted into a solidified mass upon the application of pressure, consisting in a granular mixture of bituminous material of sufficiently high penetration to be plastic at atmospheric temperatures, mineral aggregate and filler, and a surface coating of adsorbed hydrated lime on the bituminous surfaces of the individual particles.

8. A ready mixed road paving material adapted for storage in a loose condition and to be compacted into a solidified mass upon the application of pressure, consisting in a granular mixture of mineral aggregate filler, and bituminous binder material of sufficiently high penetration to be plastic at atmospheric temperatures, and a coating of finely divided calcareous material adsorbed into the bituminous surfaces of the granular particles.

JAMES F. CARLE.